# EUROPEAN PATENT SPECIFICATION

(11) **EP 0 257 580 B1**
(45) Date of publication and mention of the grant of the patent: **06.05.1992**
(21) Application number: 87112148.9
(22) Date of filing: 21.08.1987
(51) Int. Cl.: B41M 5/26

(54) **Merocyanine dye-donor element used in thermal dye transfer**
Merocyanin-Farbstoff-Donor-Element für die thermische Farbstoffübertragung
Elément donneur de colorant merocyanine utilisé pour le transfert thermique

(30) Priority: 22.08.1986 US 899274; 06.10.1986 US 915441; 08.06.1987 US 59442
(43) Date of publication of application: 02.03.1988
(73) Proprietor: EASTMAN KODAK COMPANY (a New Jersey corporation), Rochester, New York 14650 (US)
(72) Inventor: Byers, Gary Wayne, Rochester New York 14650 (US); Chapman, Derek David, Rochester New York 14650 (US)
(74) Representative: Brandes, Jürgen, Dr. rer. nat.

(56) References cited:
- EP-A- 0 257 577
- EP-A- 0 257 578
- EP-A- 0 268 179
- FR-A- 2 272 217
- PATENT ABSTRACTS OF JAPAN, vol. 10, no. 70 (M-462)[2127], 19th March 1986, page 158 M 462; & JP-A-60 214 994

## Description

This invention relates to merocyanine dye-donor elements used in thermal dye transfer which have high maximum dye densities.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta and yellow signals. The process is then repeated for the other two colors. A color hard copy is thus obtained which corresponds to the original picture viewed on a screen. Further details of this process and an apparatus for carrying it out are contained in U. S. Patent No. 4,621,271 by Brownstein entitled "Apparatus and Method for Controlling A Thermal Printer Apparatus," issued November 4, 1986.

One of the major problems in selecting a dye for thermal dye-transfer printing is to obtain good transfer efficiency to produce high maximum density. Many of the dyes proposed for use are not suitable because they yield inadequate transfer densities at reasonable coating coverages.

It is an object of this invention to provide dyes which have high transfer densities used in thermal dye-transfer printing.

Japanese Patent Publication 60/214994 relates to cyanine or merocyanine dyes which are used in an image recording material. Those dyes, however, are not used in a thermal dye transfer system. Instead, those dyes are light bleachable, such as by flash exposure, to bleach or destroy the dye. Thus, those dyes undergo substantial photolysis or decomposition when exposed to radiant energy. In addition, those dyes absorb at wavelengths substantially beyond the visible spectrum, unlike the dyes of the present invention.

EP-A- 0 257 577 (compound 4 and claim 1), EP-A- 0 257 578 (Example 2) and EP-A- 0 268 179 (Example 1) disclose a dye-donor for thermal dye transfer employing dyes similar to those claimed herein. These references, however, only constitute prior art under Article 54(3) and (4) EPC for all designated contracting states, and the relevant compounds in the prior art documents have been disclaimed.

These and other objects are achieved in accordance with the invention which comprises a dye-donor element comprising a support having thereon a dye layer characterized in that the dye comprises a merocyanine dye, other than a 3-(N-alkyl- or N-arylamino)-2-pyrazolin-5-one merocyanine dye, dispersed in a polymeric binder, the merocyanine dye being capable of transfer by diffusion to a dye-receiving element upon the application of heat, the merocyanine dye being substituted or unsubstituted on the bridging methine carbon atoms.

By appropriate selection of substituents, the merocyanine dyes employed in the invention may be of cyan, magenta or yellow hue.

In a preferred embodiment of the invention, the merocyanine dye has the formula:
wherein:
A represents -COR, -COOR, -CONHR, -CN, -SO₂R or -SO₂NR₂; or A may be combined together with R¹ to form a heterocyclic or carbocyclic ring system such as
R¹ represents -NHR, -NR₂, -OR, -SR, or -R;
n represents 0 or 1;
Z represents the atoms necessary to complete a 5- or 6-membered substituted or unsubstituted heterocyclic ring such as 3H-indole, benzoxazole, thiazoline, benzimidazole, oxazole, thiazole; and each R independently represents a substituted or unsubstituted alkyl group of from 1 to 6 carbon atoms such as methyl, ethyl, propyl, isopropyl, butyl, pentyl, hexyl or such alkyl groups substituted with hydroxy, acyloxy, alkoxy, aryl, cyano, acylamido, halogen, etc.; or a substituted or unsubstituted aryl group of from 6 to 10 carbon atoms such as phenyl, p-tolyl, m-chlorophenyl, p-methoxyphenyl, m-bromophenyl, o-tolyl, etc.

In a preferred embodiment of the invention, A and R¹ in the above formula are combined together to form the following ring system:
wherein R² is CH₃ or C₆H₅; R³ is CH₃, H or COOC₂H₅; and n is 0.

In another preferred embodiment of the invention, A and R¹ in the above formula are combined together to form the following ring system:
and n is 0.

In yet another preferred embodiment of the invention, A is -CN, n is 0 and R¹is phenyl or an alkyl group of from 1 to 6 carbon atoms.

Compounds included within the scope of the invention include the following dyes:

### Yellow Hue

### Magenta Hue

### Cyan Hue

A dye-barrier layer comprising a hydrophilic polymer may be employed in the dye-donor element of the invention between its support and the dye layer to improve the density of the transferred dye.

The dye in the dye-donor element of the invention is dispersed in a polymeric binder such as a cellulose derivative, e.g., cellulose acetate hydrogen phthalate, cellulose acetate, cellulose acetate propionate, cellulose acetate butyrate, cellulose triacetate; a polycarbonate; poly(styrene-co-acrylonitrile), a poly(sulfone) or a poly(phenylene oxide). The binder may be used at a coverage of from 0.1 to 5 g/m².

The dye layer of the dye-donor element may be coated on the support or printed thereon by a printing technique such as a gravure process.

Any material can be used as the support for the dye-donor element of the invention provided it is dimensionally stable and can withstand the heat of the thermal printing heads. Such materials include polyesters such as poly(ethylene terephthalate); polyamides; polycarbonates; glassine paper; condenser paper; cellulose esters; fluorine polymers; polyethers; polyacetals; polyolefins; and polyimides. The support generally has a thickness of from 2 to 30 µm. It may also be coated with a subbing layer, if desired.

The reverse side of the dye-donor element may be coated with a slipping layer to prevent the printing head from sticking to the dye-donor element. Such a slipping layer would comprise a lubricating material such as a surface active agent, a liquid lubricant, a solid lubricant or mixtures thereof, with or without a polymeric binder.

The dye-receiving element that is used with the dye-donor element of the invention usually comprises a support having thereon a dye image-receiving layer. The support may be a transparent film such as a poly(ether sulfone), a polyimide, a cellulose ester such as cellulose acetate, a poly(vinyl alcohol-co-acetal) or a poly(ethylene terephthalate). The support for the dye-receiving element may also be reflective such as baryta-coated paper, polyethylene-coated paper, white polyester (polyester with white pigment incorporated therein), an ivory paper, a condenser paper or a synthetic paper such as duPont Tyvek®. In a preferred embodiment, polyester with a white pigment incorporated therein is employed.

The dye image-receiving layer may comprise, for example, a polycarbonate, a polyurethane, a polyester, polyvinyl chloride, poly(styrene-co-acrylonitrile), poly(caprolactone) or mixtures thereof. The dye image-receiving layer may be present in any amount which is effective for the intended purpose. In general, good results have been obtained at a concentration of from 1 to 5 g/m².

As noted above, the dye-donor elements of the invention are used to form a dye transfer image. Such a process comprises imagewise-heating a dye-donor element as described above and transferring a dye image to a dye-receiving element to form the dye transfer image.

The dye-donor element of the invention may be used in sheet form or in a continuous roll or ribbon. If a continuous roll or ribbon is employed, it may have only the dye thereon as described above or may have alternating areas of other different dyes, such as sublimable cyan, yellow, magenta and/or black or other dyes. Such dyes are disclosed in U.S. Patent 4,541,830. Thus, one-, two-, three- or four-color elements (or higher numbers also) are included within the scope of the invention.

In a preferred embodiment of the invention, the dye-donor element comprises a poly(ethylene terephthalate) support coated with sequential repeating areas of cyan, magenta and yellow dye, at least one of the dyes being a merocyanine dye as described above, and the above process steps are sequentially performed for each color to obtain a three-color dye transfer image. Of course, when the process is only performed for a single color, then a monochrome dye transfer image is obtained.

A thermal dye transfer assemblage of the invention comprises
a) a dye-donor element as described above, and
b) a dye-receiving element as described above,
the dye-receiving element being in a superposed relationship with the dye-donor element so that the dye layer of the donor element is in contact with the dye image-receiving layer of the receiving element.

The above assemblage comprising these two elements may be preassembled as an integral unit when a monochrome image is to be obtained. This may be done by temporarily adhering the two elements together at their margins. After transfer, the dye-receiving element is then peeled apart to reveal the dye transfer image.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The following examples are provided to illustrate the invention.

### Example 1 - Preparation of Compound 1

To a suspension of 25.0 g (0.056 mole) 1,3,3-trimethyl-2-(2-N-phenylacetamidovinyl)-3-psuedo-indolium iodide in 150 mL acetonitrile were added 9.8 g (0.056 mole) 3-methyl-1-phenyl-5-pyrazolin-5-one and 10.0 mL (0.072 mole) triethylamine. The reaction was heated at reflux for 30 min., cooled to 0-5°C and the product collected by filtration and washed with cold acetonitrile. After drying in air the yield of material melting at 199-200°C was 18.7 g (93.5%). The λ-max in acetone was 476 nm.

### Example 2 - Yellow Dyes

A yellow dye-donor element was prepared by coating the following layers in the order recited on a 6 µm poly(ethylene terephthalate) support:
1) Dye-barrier layer of poly(acrylic) acid (0.16 g/m²) coated from water, and
2) Dye layer containing a yellow dye as identified in the following Table (0.63 mmoles/m²), a cellulose acetate binder (40% acetyl) at a weight equal to 1.2X that of the dye, and FC-431® (3M Corp.) surfactant (2.2 mg/m²), coated from a 2-butanone/cyclohexanone solvent mixture.
On the back side of the element was coated a typical slipping layer.

A dye-receiving element was prepared by coating a solution of Makrolon 5705® (Bayer AG Corporation) polycarbonate resin (2.9 g/m² in a methylene chloride and trichloroethylene solvent mixture on an ICI Melinex 990® white polyester support.

The dye side of the dye-donor element strip 0.75 inches (19 mm) wide was placed in contact with the dye image-receiving layer of the dye-receiver element of the same width. The assemblage was fastened in the jaws of a stepper motor driven pulling device. The assemblage was laid on top of a 0.55 (14 mm) diameter rubber roller and a TDK Thermal Head (No. L-133) and was pressed with a spring at a force of 8.0 pounds (3.6 kg) against the dye-donor element side of the assemblage pushing it against the rubber roller.

The imaging electronics were activated causing the pulling device to draw the assemblage between the printing head and roller at 0.123 inches/sec (3.1 mm/sec). Coincidentally, the resistive elements in the thermal print head were pulse-heated at increments from 0 to 8.3 msec to generate a graduated density test pattern. The voltage supplied to the print head was approximately 22v representing approximately 1.5 watts/dot (12 mjoules/dot) for maximum power.

The dye-receiving element was separated from the dye-donor element and the status A blue reflection density at the maximum density was read. The following results were obtained:

**Table 1**

| Compound | Status A Blue D-max |
|---|---|
| 1 | 1.9 |
| 2 | 1.9 |
| 3 | 1.9 |
| 4 | 1.8 |
| 5 | 1.9 |
| 6 | 2.5 |
| 7 | 2.5 |
| 9 | 1.4 |
| 10 | 1.5 |
| 37 | 1.3 |
| 38 | 1.8 |
| 39 | 1.6 |
| 40 | 2.0 |
| 41 | 2.0 |
| 42 | 2.3 |
| 43 | 1.9 |
| Control Cmpd.1 | 0.9 |
| Control Cmpd.2 | 1.1 |
| Control Cmpd.3 | 1.1 |
| Control Cmpd.4 | 0.3 |

### Yellow control compound structures:

### Control Compound 1

### Control Compound 2

### Control Compound 3

### Control Compound 4

The above results indicate that the merocyanine yellow dyes of the invention produce higher maximum density than a variety of control dyes.

### Example 3 - Magenta Dyes

Example 2 was repeated except that magenta dyes 44-46 and 48-50 were employed and the Green Status A maximum density was measured. The following results were obtained:

**Table 2**

| Compound | Status A Green D-max |
|---|---|
| 44 | 2.5 |
| 45 | 2.8 |
| 46 | 2.7 |
| 48 | 1.9 |
| 49 | 1.8 |
| 50 | 1.6 |
| Control Cmpd.5 | 0.6 |
| Control Cmpd.6 | 1.6 |

### Magenta control compound structures:

### Control Compound 5

Described in JP 60/253,595.

### Control Compound 6

Described in JP 60/159,091.

The above results indicate that with one exception, the merocyanine magenta dyes of the invention produce higher maximum density than prior art magenta anthraquinone control dyes.

### Example 4 - Cyan Dyes

Example 2 was repeated except that cyan dyes 51-53 were employed and the Red Status A maximum density was measured. The following results were obtained:

**Table 3**

| Compound | Status A Red D-max |
|---|---|
| 51 | 1.7 |
| 52 | 1.3 |
| 53 | 2.1 |
| Control Cmpd.7 | 1.2 |
| Control Cmpd.8 | 0.6 |

### Cyan control compound structures:

### Control Compound 7

Described in JP 60/172,591.

### Control Compound 8

Described in JP 60/151,097 and JP 61/035,993.

The above results indicate that the merocyanine cyan dyes of the invention produce higher maximum density than prior art anthraquinone cyan control dyes.

## Claims

1. A dye-donor element for thermal dye transfer comprising a support having thereon a dye layer, characterized in that the dye comprises a merocyanine dye, other than a 3-(N-alkyl- or N-arylamino)-2-pyrazolin-5-one merocyanine dye, dispersed in a polymeric binder, said merocyanine dye being capable of transfer by diffusion to a dye-receiving element upon the application of heat, said merocyanine dye being substituted or unsubstituted on the bridging methine carbon atoms.

2. The element of Claim 1 characterized in that said merocyanine dye has the formula: wherein:
A represents -COR, -COOR, -CONHR, -CN, -SO₂R or -SO₂NR₂; or A may be combined together with R¹ to form a heterocyclic or carbocyclic ring system;
R¹ represents -NHR, -NR₂, -OR, -SR, or -R;
n represents 0 or 1;
Z represents the atoms necessary to complete a 5- or 6-membered substituted or unsubstituted heterocyclic ring; and
each R independently represents a substituted or unsubstituted alkyl group of from 1 to 6 carbon atoms or a substituted or unsubstituted aryl group of from 6 to 10 carbon atoms.

3. The element of Claim 2 characterized in that A and R¹ are combined together to form the following ring system: wherein R² is CH₃ or C₆H₅; R³ is CH₃, H or COOC₂H₅; and n is 0.

4. The element of Claim 2 characterized in that A and R¹ are combined together to form the following ring system: and n is 0.

5. The element of Claim 2 characterized in that A is -CN, n is 0 and R¹ is phenyl or an alkyl group of from 1 to 6 carbon atoms.

6. The element of Claim 1 wherein said support comprises poly(ethylene terephthalate), said dye layer comprises sequential repeating areas of cyan, magenta and yellow dye, and at least one of said dyes being said merocyanine dye.

7. A thermal dye transfer assemblage comprising:
a) a dye-donor element comprising a support having thereon a dye layer comprising a dye dispersed in a polymeric binder, and
b) a dye-receiving element comprising a support having thereon a dye image-receiving layer,
said dye-receiving element being in a superposed relationship with said dye-donor element so that said dye layer is in contact with said dye image-receiving layer,
characterized in that said dye comprised a merocyanine dye, other than a 3-(N-alkyl- or N-aryl-amino)-2-pyrazolin-5-one merocyanine dye, which is capable of transfer by diffusion to a dye-receiving element upon the application of heat, said merocyanine dye being substituted or unsubstituted on the bridging methine carbon atoms.

8. The assemblage of Claim 7 characterized in that said merocyanine dye has the formula: wherein:
A represents -COR, -COOR, -CONHR, -CN, -SO₂R or -SO₂NR₂; or A may be combined together with R¹ to form a heterocyclic or carbocyclic ring system;
R¹ represents -NHR, -NR₂, -OR, -SR, or -R;
n represents 0 or 1;
Z represents the atoms necessary to complete a 5- or 6-membered substituted or unsubstituted heterocyclic ring; and
each R independently represents a substituted or unsubstituted alkyl group of from 1 to 6 carbon atoms or a substituted or unsubstituted aryl group of from 6 to 10 carbon atoms.

9. The assemblage of Claim 8 characterized in that A and R¹ are combined together to form the following ring system: wherein R² is CH₃ or C₆H₅; R³ is CH₃, H or COOC₂H₅; and n is 0.

10. The assemblage of Claim 8 characterized in that A and R¹ are combined together to form the following ring system; and n is 0.

11. The assemblage of Claim 8 characterized in that A is -CN, n is 0 and R¹ is phenyl or an alkyl group of from 1 to 6 carbon atoms.

## Revendications

1. Elément donneur de colorant pour transfert de colorant par la chaleur comprenant un support recouvert d'une couche de colorant, caractérisé en ce que le colorant comprend un colorant mérocyanine, autre qu'un colorant 3-(N-alkyl- ou N-aryl amino)-2-pyrazolin-5-one, dispersé dans un liant polymère, le colorant mérocyanine étant susceptible d'être transféré par diffusion sur un élément récepteur de colorant par application de la chaleur, le colorant mérocyanine étant substitué ou non sur les atomes de carbone de la liaison méthine.

2. Elément selon la revendication 1 caractérisé en ce que le colorant mérocyanine a la formule : où
A représente -COR, -COOR, -CONHR, -CN, -SO₂R ou -SO₂NR₂ ; ou A peut être combiné avec R¹ pour former un système cyclique hétérocyclique ou carbocyclique ;
R¹ représente -NHR, -NR₂, -OR, -SR, ou -R ;
n représente 0 ou 1 ;
Z représente le nombre d'atomes nécessaire pour compléter un hétérocycle substitué ou non à 5 ou 6 chaînons ; et
chaque R séparément représente un groupe alkyle substitué ou non de 1 à 6 atomes de carbone ou un groupe aryle substitué ou non de 6 à 10 atomes de carbone.

3. Elément selon la revendication 2 caractérisé en ce que A et R¹ sont combinés ensemble pour former le système cyclique suivant : où R² est CH₃ ou C₆H₅ ; R³ est CH₃, H ou COOC₂H₅ ; et n est 0.

4. Elément selon la revendication 2 caractérisé en ce que A et R¹ sont combinés ensemble pour former le système cyclique suivant : et n est 0.

5. Elément selon la revendication 2 caractérisé en ce que A est -CN, n est 0 et R¹ est un groupe phényle ou alkyle de 1 à 6 atomes de carbone.

6. Elément selon la revendication 1 caractérisé en ce que le support est en polytéréphtalate d'éthylène, la couche de colorant comprend des séquences répétitives de zones de colorants cyan, magenta et jaune et au moins un des colorants est le colorant mérocyanine.

7. Assemblage pour transfert de colorant par la chaleur comprenant :
a) un élément donneur de colorant comprenant un support recouvert d'une couche de colorant comprenant un colorant dispersé dans un liant polymère, et
b) un élément récepteur de colorant comprenant un support recouvert d'une couche réceptrice d'image de colorant,
l'élément récepteur de colorant et l'élément donneur de colorant étant superposés de telle sorte que la couche de colorant est en contact avec la couche réceptrice d'image de colorant,
caractérisé en ce que le colorant comprend un colorant mérocyanine, autre qu'un colorant 3-(N-alkyl- ou N-aryl amino)-2-pyrazolin-5-one,
qui est susceptible d'être transféré sur un élément récepteur de colorant par application de la chaleur et est substitué ou non sur les atomes de carbone de la liaison méthine.

8. Assemblage selon la revendication 7 caractérisé en ce que le colorant mérocyanine a la formule : où
A représente -COR, -COOR, -CONHR, -CN, -SO₂R ou -SO₂NR₂ ; ou A peut être combiné avec R¹ pour former un système cyclique hétérocyclique ou carbocyclique ;
R¹ représente -NHR, -NR₂, -OR, -SR, ou -R ;
n représente 0 ou 1 ;
Z représente le nombre d'atomes nécessaire pour compléter un hétérocycle substitué ou non à 5 ou 6 chaînons ; et
chaque R séparément représente un groupe alkyle substitué ou non de 1 à 6 atomes de carbone ou un groupe aryle substitué ou non de 6 à 10 atomes de carbone.

9. Assemblage selon la revendication 8 caractérisé en ce que A et R¹ sont combinés ensemble pour former le système cyclique suivant : où R² est CH₃ ou C₆H₅ ; R³ est CH₃, H ou COOC₂H₅ ; et n est 0.

10. Assemblage selon la revendication 8 caractérisé en ce que A et R¹ sont combinés ensemble pour former le système cyclique suivant : et n est 0.

11. Assemblage selon la revendication 8 caractérisé en ce que A est -CN, n est 0 et R¹ est un groupe phényle ou alkyle de 1 à 6 atomes de carbone.

## Patentansprüche

1. Farbstoff-Donorelement für die thermische Farbstoffübertragung mit einem Träger, auf dem sich eine Farbstoffschicht befindet, dadurch gekennzeichnet, daß der Farbstoff einen Merocyaninfarbstoff umfaßt, der von einem 3-(N-Alkyl- oder N-Aryl-amino)-2-pyrazolin-5-on-Merocyaninfarbstoff verschieden ist, und in einem polymeren Bindemittel dispergiert vorliegt, wobei der Merocyaninfarbstoff bei Einwirkung von Wärme durch Diffusion auf ein Farbstoff-Empfangselement übertragbar ist, und wobei der Merocyaninfarbstoff an den brückenbildenden Methin-Kohlenstoffatomen substituiert oder unsubstituiert ist.

2. Element nach Anspruch 1, dadurch gekennzeichnet, daß der Merocyaninfarbstoff der Formel: entspricht, in der bedeuten:
A gleich -COR, -COOR, -CONHR, -CN,-SO₂R oder -SO₂NR₂; oder gemeinsam mit R¹ ein heterocyclisches oder carbocyclisches Ringsystem;
R¹ gleich -NHR, -NR₂, -OR, -SR, oder -R;
n gleich 0 oder 1;
Z die Atome, die zur Vervollständigung eines 5- oder 6-gliedrigen substituierten oder unsubstituierten heterocyclischen Ringes erforderlich sind; und
R jeweils unabhängig voneinander eine substituierte oder unsubstituierte Alkylgruppe mit 1 bis 6 Kohlenstoffatomen oder eine substituierte oder unsubstituierte Arylgruppe mit 6 bis 10 Kohlenstoffatomen.

3. Element nach Anspruch 2, dadurch gekennzeichnet, daß A und R¹ gemeinsam das folgende Ringsystem bilden: in dem R² für -CH₃ oder -C₆H₅ steht; R³ gleich -CH₃, -H oder -COOC₂H₅ ist und n für 0 steht.

4. Element nach Anspruch 2, dadurch gekennzeichnet, daß A und R¹ gemeinsam das folgende Ringsystem bilden: und n gleich 0 ist.

5. Element nach Anspruch 2, dadurch gekennzeichnet, daß A für -CN steht, n gleich 0 ist und R¹ die Bedeutung einer Phenyl- oder einer Alkylgruppe mit 1 bis 6 Kohlenstoffatomen hat.

6. Element nach Anspruch 1, in dem der Träger ein Poly(ethylenterephthalat)träger ist und die Farbstoffschicht in Folge wiederkehrende Bereiche von blaugrünem, purpurrotem und gelbem Farbstoff aufweist und mindestens einer der Farbstoffe der Merocyaninfarbstoff ist.

7. Einheit für die thermische Farbstoffübertragung mit:
a) einem Farbstoff-Donorelement mit einem Träger, auf dem sich eine Farbstoffschicht mit einem in einem polymeren Bindemittel dispergierten Farbstoff befindet, und
b) einem Farbstoff-Empfangselement mit einem Träger, auf dem eine Farbbild-Empfangsschicht angeordnet ist,
wobei das Farbstoff-Empfangselement dem Farbstoff-Donorelement überlagert ist, so daß sich die Farbstoffschicht in Kontakt mit der Farbbildempfangsschicht befindet, dadurch gekennzeichnet, daß der Farbstoff einen Merocyaninfarbstoff umfaßt, der von einem 3-(N-Alkyl- oder N-Aryl-amino)-2-pyrazolin-5-on-Merocyaninfarbstoff verschieden ist, und in einem polymeren Bindemittel dispergiert vorliegt, wobei der Merocyaninfarbstoff bei Einwirkung von Wärme durch Diffusion auf ein Farbstoff-Empfangselement übertragbar ist, und wobei der Merocyaninfarbstoff an den brückenbildenden Methin-Kohlenstoffatomen substituiert oder unsubstituiert ist.

8. Einheit nach Anspruch 7, dadurch gekennzeichnet, daß der Merocyaninfarbstoff der Formel: entspricht, in der bedeuten:
A gleich -COR, -COOR, -CONHR, -CN,-SO₂R oder -SO₂NR₂; oder gemeinsam mit R¹ ein heterocyclisches oder carbocyclisches Ringsystem;
R¹ gleich -NHR, -NR₂, -OR, -SR, oder -R;
n gleich 0 oder 1;
Z die Atome, die zur Vervollständigung eines 5- oder 6-gliedrigen substituierten oder unsubstituierten heterocyclischen Ringes erforderlich sind; und
R jeweils unabhängig voneinander eine substituierte oder unsubstituierte Alkylgruppe mit 1 bis 6 Kohlenstoffatomen oder eine substituierte oder unsubstituierte Arylgruppe mit 6 bis 10 Kohlenstoffatomen.

9. Einheit nach Anspruch 8, dadurch gekennzeichnet, daß A und R¹ gemeinsam das folgende Ringsystem bilden: in dem R² für -CH₃ oder -C₆H₅ steht; R³ gleich -CH₃, -H oder -COOC₂H₅ ist und n für 0 steht.

10. Einheit nach Anspruch 8, dadurch gekennzeichnet, daß A und R¹ gemeinsam das folgende Ringsystem bilden: und n gleich 0 ist.

11. Einheit nach Anspruch 8, dadurch gekennzeichnet, daß A für -CN steht, n gleich 0 ist und R¹ die Bedeutung einer Phenyl- oder einer Alkylgruppe mit 1 bis 6 Kohlenstoffatomen hat.
